

Patented Sept 19, 1939

T347  
2,173,824

## UNITED STATES PATENT OFFICE

2,173,824

## COMPOSITION FOR PRINTING TEXTILE FIBERS

Ivan F. Chambers, Wilmington, Del., assignor to  
E. I. du Pont de Nemours & Company, Wilmington, Del., a corporation of DelawareNo Drawing. Application March 17, 1937,  
Serial No. 131,525

6 Claims. (Cl. 8—70)

This invention pertains to an improved process for printing textile fibers and fabrics with vat dyes, and to vat dye compositions especially adapted for such purposes. More particularly it relates to the preparation of printing compositions containing a vat dyestuff and a material adapted to facilitate the printing operation. Still more particularly it relates to the preparation of printing pastes which contain materials adapted to facilitate the penetration of the dye during a printing operation. Still more particularly it relates to the printing of fabrics composed of natural or artificial or mixed fibers, and particularly lustrous or delustered regenerated cellulose fibers, with pastes containing agents which facilitate the printing operation. In a more limited sense it relates to vat dye powders or pastes containing agents which give improved penetration and levelness, and to fabrics printed with the above compositions.

By the term "vat dyestuff" as used hereinafter I refer to dyestuffs such as those of the anthraquinone, indigo, thioindigo and sulfur series which are capable of being reduced by the aid of alkaline hydrosulfite.

The fixation of vat colors on textile fabrics by reduction and subsequent oxidation is one of the most important dyeing procedures in the textile field. In calico printing, the reduction is effected partially or wholly when the printed material is subjected to the action of steam. During the steaming or aging operation the dyestuff is mechanically held on the cloth by a vehicle consisting of a starch, dextrin or other paste.

Printing compositions may contain the vat dyestuff in its oxidized form or its reduced, that is, the leuco form. A suitable printing composition may be prepared by mixing the dyestuff paste with a thickening containing an alkaline reacting substance and a reducing agent. As examples of alkaline reacting substances may be mentioned potassium carbonate, sodium carbonate and sodium hydroxide. The reducing agents referred to may be an alkali metal aldehyde sulfoxylate, alkali metal hydrosulfite or glucose. The usual thickening agents are British gum (dextrin), starch and/or gum tragacanth. A small percentage of glycerin is usually added to the printing composition as an assistant.

Processes are also known which employ stabilized water-soluble forms of the vat dyestuffs, such as the leuco-esters of the vat dyestuff, known as "Indigosol" colors. These colors are water-soluble and require no reducing agent.

Application consists in impregnating the fabric with the color and fixing the dyestuff on the fiber by subsequent hydrolysis and oxidation.

In the processes just described and others, special assistants are generally added to the dyestuff composition or printing paste, to facilitate the dispersion of the dyestuff, penetration, reduction, oxidation, etc. The state of perfection, however, has not yet been attained, and the printer generally has to cope with such problems as poor penetration of the color into the fiber, low tintorial yield, lack of brilliancy in the prints, specky or mottled prints. He is also quite restricted in the conditions of operation, and will frequently obtain inferior results if the aging time is curtailed or if the percentage of reducing agent in the printing composition is appreciably reduced. In printing with the water-soluble forms of the vat dyestuffs, the additional problem enters of obtaining deep shades. Light shades are, as a rule, obtained readily with leuco-esters but only a few of the latter have sufficient solubility and penetrating power to produce a satisfactory deep shade.

It is an object of this invention to provide a process for printing with vat dyestuffs which is characterized by the production of uniform prints, free from speckiness, and of good penetration. It is a further object of this invention to produce novel dyestuff compositions and/or printing pastes which are particularly adapted for the process aforementioned. It is a still further object of this invention to provide novel vat dyestuff compositions which possess good wetting, penetrating and dispersing power, and permit of efficient utilization of the color. A still further object of this invention is to produce vat dye powders or grains which are essentially non-hygroscopic and which possess good wetting, penetrating and dispersing power. A still further object is to produce prints of exceptional strength, brilliancy, penetration on natural and particularly on lustrous and delustered regenerated cellulose fibers. Another object is to produce dyeings of exceptional levelness, penetration, strength and brilliancy by the pigment-pad method or by continuous or intermittent machine method. Other and further objects of this invention will appear hereinafter.

These and other objects are accomplished by incorporating into a dyestuff composition benzyl alcohol. In a more limited sense they are accomplished by incorporating into a printing paste, directly or by way of first mixing with the vat dyestuff, benzyl alcohol. In a still more limited sense they are accomplished by incorporating into a dye composition containing a printing assistant, and more particularly a printing assistant having wetting properties, benzyl alcohol.

While good results are obtained when benzyl

alcohol is added to any printing composition containing a dyeing ingredient, improved results are obtained if a sulfonated textile assistant having wetting and dispersing properties is added to the composition together with the benzyl alcohol. Excellent results are obtained if the sulfonated textile assistant is Turkey red oil and/or a water-soluble alcohol sulfate having from six to twelve carbon atoms in which the radical attached to the sulfate group contains a straight chain of not more than six carbon atoms.

In the preferred embodiment of the invention, they are accomplished by incorporating into a printing paste, directly or by way of first mixing with the dyestuff, a mixture of assistants of the following general composition:

|                                                                         | Per cent            |
|-------------------------------------------------------------------------|---------------------|
| Benzyl alcohol                                                          | 0.1 to 20           |
| Turkey red oil                                                          | 1.0 to 40           |
| 20 One or more water-soluble alcohol sulfates as subsequently described | 1.0 to 40           |
| Diluent such as water, British gum, starch, sugar, glucose, etc.        | 97.9 to 0           |
| 25                                                                      | <u>100.0 to 100</u> |

Each of the components of the above mixture exerts a specific assistant effect in that one component cannot be successfully substituted for another component. The collective assistant effect obtained from the mixture is more advantageous for our purpose than the effect obtained from the individual components.

35 The water-soluble alcohol sulfates referred to above contain not less than six and up to twelve carbon atoms per molecule, but in which the radical attached to the sulfate group does not contain a straight chain of more than six  $\text{CH}_2$  groups.

Typical and most available compounds of the above general definition are the mono-sodium-sulfates of the higher alcohols obtained as by-products in the synthetic manufacture of methanol. The latter process generally involves catalytic hydrogenation of mixtures of carbon monoxide and carbon dioxide. But in addition to the main desirable product, methanol, and in addition to other organic compounds of low molecular weight, such as ketones and alcohols below amyl, there is generally obtained a series of by-product branched alcohols, having a total of from seven to twelve carbon atoms. These alcohols are usually not isolated individually, nor is such individual isolation necessary for the purpose of this invention. Instead, the entire mass of by-products is separated into fractions according to boiling point.

60 The fractions which I found most useful for the purpose of this invention have, as alcohols, the following boiling ranges and dominant composition. For the sake of facility, I shall herein designate them and later refer to them as fractions A, B, C and D.

| Fraction | Boiling range                  | Alcohols dominant in the fraction                                 |
|----------|--------------------------------|-------------------------------------------------------------------|
| 70 A     | $^{\circ}\text{C.}$<br>133-150 | Mixture of $\text{C}_6$ primary and $\text{C}_7$ secondary.       |
| B        | 150-160                        | Mixture of $\text{C}_7$ primary and $\text{C}_8$ secondary.       |
| C        | 160-200                        | Mixture of $\text{C}_8-\text{C}_{10}$ both primary and secondary. |
| D        | 200-260                        | Mixture of $\text{C}_{10}$ and above, primary and secondary.      |

However, I named these fractions above as the preferred compounds for my invention merely because of their ready availability and cheapness. If available, the individual constituents of the above fractions may be used in pure form. As 5 typical compounds of this series may be mentioned the following individual compounds or mixtures thereof: 4-methyl-1-pentanol; 2-methyl-1-pentanol; 2,4-dimethyl-1-pentanol; 3-methyl-2-pentanol; 2,4-dimethyl-3-pentanol (di-isopropyl-carbinol); 2-methyl-3-pentanol; 4-methyl-1-hexanol; 2,4-dimethyl-1-hexanol; 2,5-dimethyl-3-hexanol; and numerous others. 10

It will be noted that the parent alcohols may be primary or secondary. It will be noted further 15 that they are all characterized by containing no long chains at all, or else containing a long chain loaded with side chains.

I found that best results are obtained with compounds wherein the direct chain between the 20 sulfated alcohol function and the nearest branching point is not longer than four, or at most six carbon atoms.

As for the sulfate group, it may be neutralized by a cation which does not impair the water-solubilizing tendencies of the sulfate function. 25 Such cations are the alkali metals, for instance sodium or potassium, and water-soluble organic bases, especially those which contain free OH groups or other groups conferring water-solubility. Examples of such organic bases are the mono-, di- or tri-alkylamines, mono-, di- or tri-ethanolamine, the corresponding propanolamines, the butanolamines, cyclohexylamine, cyclohexyl-mono- or di-ethanolamine, dimethylethanolamine, n-butyramine, guanidine, tetraethylammonium hydroxide, glucamine, n-methyl-glucamine, diglycerylamine, 1,3-diamino-n-propanol, 1-amino-propane-diol, etc. 30 35

My invention does not require the use of the 40 above novel assistants exclusively, but on the contrary other assistants of the customary and well known types may be added, and indeed are often very desirable. These subsidiary assistants may be incorporated into the eventual printing 45 paste in any desirable manner. For instance, they may be mixed with the benzyl alcohol of this invention to produce an assistant preparation for the convenient use of the printer. Or they may be incorporated by the dyestuff manufacturer 50 jointly with the benzyl alcohol or mixtures of the same with sulfonated textile assistants having wetting and dispersing properties, directly into the dyestuff preparation, to be marketed thus as a color preparation especially suited for printing. 55 Or one of the assistants may be incorporated into the dyestuff while the other is incorporated into the thickening paste or reducing preparation eventually mixed with the dyestuff.

Among these additional or subsidiary assistants 60 may be mentioned wetting and dispersing agents, reducing agents, reducing catalysts, emulsifying agents, lubricants, inert solid or liquid diluents, etc. The individual representatives of these various classes are well known in the art 65 of printing, and it will be sufficient for the purpose of illustration to name here but a few typical members: for instance, sodium benzyl sulfonilate, isopropyl-naphthalene sodium sulfonate, diethylene glycol, sodium oleate, pine oil, glucose, sucrose, dextrose, sodium carbonate, sodium hydrosulfite, sodium sulfoxylate formaldehyde, hydroxy-alkylamines, tetralin sodium sulfonate, tetralin, hexalin, glycerin, etc. As sub- 70 75

8. BLEACHING & DYEING; FLUID TREATMENT & CHEMICAL MODIFICATION OF TEXTILES & FIBERS,

70

2,173,824

3

5 subsidiary assistants not heretofore commonly employed in this art may be mentioned the free alcohols corresponding to the sulfates of this invention, especially the methanol by-products above mentioned, and the carboxylic acids obtained by the oxidation of these fractions, as more particularly described in U. S. Patent 1,856,263 and copending application of Hans C. Duus, Serial No. 735,297.

10 The sulfuric acid esters or sulfates of the above defined alcohols, forming the major object of this invention, may be prepared in well known manner. A convenient and practically universal method is to react the corresponding alcohol with

15 from 65% to 100% of theory (based on the hydroxyl number) of chlorosulfonic acid, and then neutralizing with the desired inorganic or organic base. The resulting aqueous solution may be used directly, without troubling to isolate the 20 alkylsulfate. The residual free alcohol, where a deficiency of chlorosulfonic acid is employed, is not a detriment, as has already been indicated.

The concentration of the new assistant mixture and the method of application may vary 25 within wide limits depending on the desired results or convenience. The following general procedures may be used:

(a) Addition of an aqueous solution or stable emulsion to the printing composition;

30 (b) Addition of a dry assistant mixture to the printing composition;

(c) Addition of a dry assistant mixture containing a diluent such as sugar, starch, glucose, or British gum;

35 (d) Preparation of an assistant color paste whereby the vat color pigment or leuco sulfuric ester derivative is intimately mixed with an aqueous solution or stable emulsion;

(e) Preparation of an assistant color powder 40 whereby the vat color pigment is intimately mixed with a dry assistant mixture and/or an inert diluent such as sugar, starch, glucose, or British gum.

The proportion of assistant with respect to 45 the weight of the printing paste may likewise vary within wide limits, good results being obtained with proportions from 0.1 to 20.0%, and preferably from 5 to 20%, depending on the composition used.

50 Where these assistants are incorporated in the marketable dye composition, the latter may be prepared in paste form or dry, for instance powder, grains or flakes, with suitable diluents such as sugar, starch, glucose, British gum, etc., as 55 most convenient.

Without limiting this invention the following examples are given to illustrate my preferred mode of operation. Parts are by weight.

60 **EXAMPLE I**

Illustrating preparation of the thickening pastes.

65 **Thickening SBG**

100 parts of wheat starch and  
300 parts of British gum were pasted with  
600 parts of water

70 —  
1000 parts

This mixture was heated at the boil for ten minutes and cooled to room temperature. A 75 smooth paste was obtained.

**Thickener A**

560 parts of Thickening SBG were heated to 170° F. There were then added  
170 parts of potassium carbonate. After the 5 potassium carbonate had dissolved, the paste was cooled to 140° F. and the following ingredients added  
120 parts of sodium sulfoxylate formaldehyde  
50 parts of glycerin  
100 parts of water

1000 parts

The whole was stirred to form a smooth paste.

15

**Thickener B**

550 parts of Thickening SBG  
50 parts of potassium carbonate  
250 parts of caustic soda (35% solution)  
150 parts of glucose

1000 parts

**Thickener C**

520 parts of Thickening SBG were heated to 25 170° F. There were then added  
200 parts of potassium carbonate. The paste was cooled to 140° F. and the following ingredients added  
180 parts of sodium sulfoxylate formaldehyde  
50 parts of glycerin  
50 parts of water

1000 parts

35

The following examples illustrate the preferred embodiment of my invention.

**EXAMPLE II**

20 parts of "Sulfanthrene" Orange R Paste (Color Index #1222) were mixed with  
78 parts of Thickener A. To this were added  
2 parts of benzyl alcohol

100 parts

45

Lustrous and titanium dioxide delustered rayon piece goods were printed with the above printing composition, dried and aged for five minutes at 214° F. in a rapid ager of the Mather 50 Platt type. The printed material was then treated for one minute in an oxidizing bath at 140° F. containing 0.5% of sodium bichromate and 0.5% of acetic acid, rinsed in cold water, soaped for five minutes in a soap bath at 160° F. containing 55 0.5% of soap, rinsed and dried. Bright orange prints of exceptional penetration were obtained.

In the above example, the dyestuff may be replaced by any other vat dye of the indigoid, thio-indigoid or anthraquinone series, as for instance, 60 "Ponsol" Dark Blue BR Paste (Color Index #1099), "Sulfanthrene" Blue 2BD Double Paste (Color Index #1184), "Sulfanthrene" Pink FF Paste (Color Index #1211), "Sulfanthrene" Violet B Double Paste (Color Index #1222), 65 "Ponsol" Yellow G Double Paste (Color Index #1118), "Sulfanthrene" Yellow R Paste (Color Index #1170), "Ponsol" Brown AR Double Paste (Color Index #1151), "Ponsol" Blue GD Double Paste (Color Index #1113), "Ponsol" Golden 70 Orange G Double Paste (Color Index #1096), "Ponsol" Flavone GC Paste (Color Index #1095), "Ponsol" Blue BCS Double Paste (Color Index #1114), "Ponsol" Jade Green Paste (Color Index #1101), and many others.

75

## EXAMPLE III

20 parts of "Ponsol" Jade Green Paste (Color Index #1101) were mixed with  
 70 parts of Thickener C. To this were added  
 5 1 part of benzyl alcohol and  
   9 parts of Turkey red oil  
 100 parts

10 Lustrous and ethylene glycol di-beta-naphthyl ether delustered rayon piece goods were printed with the above printing composition, dried, aged, and developed as in Example II. A bright green print of exceptional uniformity and penetration was obtained.

## EXAMPLE IV

15 parts of "Sulfanthrene" Blue 2BD Double Paste (Color Index #1184) were mixed with  
 20 60 parts of Thickener A as prepared in Example I  
 14 parts of Thickening SBG  
 3 parts of sodium hydrosulfite and  
 25 8 parts of a stable emulsion consisting of  
   25 parts of isopropyl naphthalene sodium sulfonate  
   60 parts of water and  
   15 parts of benzyl alcohol  
 30 100 parts

100 parts

The printing paste was heated to 140° F. during which the color was reduced to a considerable extent and then cooled to room temperature. Piece goods containing viscose rayon, Bemberg rayon, cellulose acetate rayon, and titanium dioxide delustered rayon fibers were printed with the above printing composition, dried and aged for five minutes at 218° F. After aging the print was immersed for two minutes in a bath at 130° F. containing 0.5% of sodium perborate and 0.5% of acetic acid. A brilliant blue dyeing of exceptional levelness and penetration on all types of fibers was obtained.

## EXAMPLE V

20 parts of "Ponsol" Brilliant Violet RR Paste were mixed with  
 50 70 parts of Thickener C. To this were added  
 10 parts of a solution consisting of  
   85 parts of diethylene glycol  
   15 parts of benzyl alcohol  
 55 100 parts

100 parts

Piece goods containing cotton, viscose rayon, cuprammonium rayon, and barium sulfate delustered viscose rayon fibers were printed with the above printing paste, dried and aged for five minutes at 216° F. The print was then developed as in Example II. A bright level violet print of exceptional color value and penetration was obtained.

## EXAMPLE VI

5 parts of "Sulfogene" Fast Black CL (Indo-carbon CL) were mixed with  
 70 5 parts of glycerin. To this was added  
 80 parts of Thickener B as in Example I  
   3 parts of benzyl alcohol and  
   7 parts of Turkey red oil  
 75 100 parts

Cotton, lustrous rayon, and titanium dioxide delustered rayon were printed with the above printing composition, dried, aged for five minutes at 214° F. and developed as in Example II. A brilliant and uniform print of excellent penetration to the reverse side of the fabric was obtained.

## EXAMPLE VII

5 parts of Indigosol O4B (Leuco sulfuric ester derived from Ciba Blue 2BD—Color Index #1184) were mixed with  
 5 parts of Cellosolve (ethylene-glycol-mono-ethyl-ether)  
 2 parts of benzyl alcohol  
 20 parts of warm water (160° F.) and  
 58 parts of neutral starch tragacanth thickening. There were then added  
 4 parts of ammonium sulfocyanide (50% solution)  
 4 parts of sodium chlorate (23% solution)  
 1 part of ammonium vanadate (1% solution)  
 1 part of ammonia (25% solution)  
 100 parts

15  
 20  
 25  
 25

## Starch tragacanth thickening

100 parts of wheat starch  
 360 parts of gum tragacanth (6% solution)  
 540 parts of water

30

1000 parts

Heated at the boil for 15 minutes, cooled.

Piece goods containing cotton, lustrous and titanium dioxide delustered rayon were printed with the above printing composition, dried, and aged for six minutes in the rapid ager. After aging the material was rinsed, soaped for five minutes at 160° F. in a 0.5% soap solution, rinsed, and dried. A brilliant level blue dyeing showing exceptional penetration of color to the reverse side of the fabric was obtained.

## EXAMPLE VIII

100 parts of "Sulfanthrene" Orange R Paste (Color Index #1217) were mixed with  
 10 parts of benzyl alcohol  
 110 parts. There were then evaporated  
 10 parts of water producing

50

100 parts of Assistant "Sulfanthrene" Orange R Paste

55

The above was milled in a colloid mill producing a finely dispersed assistant dyestuff paste adapted for handling in commerce.

## EXAMPLE IX

100 parts of "Ponsol" Blue GD Double Paste (Color Index #1113) were mixed with  
 50 parts of Turkey red oil and  
 12 parts of benzyl alcohol  
 162 parts. There were then evaporated  
 62 parts of water producing

65

100 parts of Assistant "Ponsol" Blue GD Double Paste

70

The above was milled for one hour in a rod mill producing a finely dispersed assistant dyestuff paste, especially suitable for printing rayon.

75

8. BLEACHING & DYEING; FLUID  
TREATMENT & CHEMICAL MODIFI-  
CATION OF TEXTILES & FIBERS.

Search Room

70

2,173,824

5

EXAMPLE X

20 parts of "Sulfanthrene" Orange R Paste (Color Index #1222) were mixed with  
5 79 parts of Thickener A. There were then added  
10 parts of a stable emulsion consisting of  
30 parts of Turkey red oil  
60 parts of Assistant A (described  
below) and  
10 10 parts of benzyl alcohol  
100 parts  
100 parts

15 Fabrics containing (a) cotton and lustrous viscose rayon, (b) lustrous and titanium dioxide delustered viscose rayon, (c) lustrous and titanium dioxide delustered cellulose acetate rayon were printed with the above printing composition, dried, and aged for five minutes at 214° F. in a rapid ager of the Mather Platt type. The printed materials were then treated for one minute in an oxidizing bath at 140° F. containing 0.5% of sodium bichromate and 0.5% of acetic acid, rinsed in cold water, soaped for five minutes in a soap bath at 160° F. containing 0.5% of soap, rinsed, and dried. Brilliant level prints were obtained on all fabrics according to the pattern of the 20 printing roll. The prints were very sharp in outline and showed exceptionally good penetration to the reverse side of the fabrics.

In the above example, Assistant A is a 30% aqueous solution of mixed sodium alkyl sulfates obtained by the sulfation of a mixture of C<sub>6</sub> primary and C<sub>7</sub> secondary alcohols (B. P. 133°-150° C.).

Assistant A may be substituted with equally good results by Assistants B, C or D, as described 40 below. Assistant B is a 30% aqueous solution of mixed sodium alkyl sulfates obtained by the sulfation of a mixture of C<sub>7</sub> primary and C<sub>8</sub> secondary alcohols (B. P. 150°-160° C.).

Assistant C is a 30% aqueous solution of mixed 45 sodium alkyl sulfates obtained by the sulfation of a mixture of C<sub>8</sub> to C<sub>10</sub> primary and secondary alcohols (B. P. 160°-200° C.).

Assistant D is a 30% aqueous solution of mixed 50 sodium alkyl sulfates obtained by the sulfation of a mixture of C<sub>10</sub> and above, primary and secondary alcohols (B. P. 200°-260° C.).

In the above example, the dyestuffs may be replaced by other vat colors of the indigoid, thio-indigoid, or anthraquinone series, for instance 55 "Sulfanthrene" Red 3B Paste (Color Index #1212), "Sulfanthrene" Blue 2BD Paste (Color Index #1184), "Sulfanthrene" Violet B Paste (Color Index #1222), "Sulfanthrene" Pink FF Paste (Color Index #1211), "Sulfanthrene" Scarlet Y Paste (Color Index #1228), "Sulfanthrene" Yellow R Paste (Color Index #1170), "Sulfanthrene" Brown G Paste (or Ciba Brown G Paste), "Ponsol" Blue GD Double Paste (Color Index #1113), "Ponsol" Flavone GC Paste (Color Index #1095), "Ponsol" Jade Green Paste (Color Index #1101), "Ponsol" Golden Orange G Double Paste (Color Index #1096), "Ponsol" Brown AR Double Paste (Color Index #1151), "Ponsol" 65 Yellow G Double Paste (Color Index #1118), "Ponsol" Blue BCS Double Paste (Color Index #1114), "Ponsol" Dark Blue BR Paste (Color Index #1099), "Ponsol" Violet RRD Paste (Color Index #1104), "Ponsol" Blue Green FFB Double Paste (Color Index #1173), and many others.

EXAMPLE XI

50 parts of "Ponsol" Dark Blue BR (Color Index #1099) press cake containing 26% color solids were mixed with  
1 part of formaldehyde-naphthalene sulfonic acid condensation product (30% solution)  
40 parts of diethylene glycol and  
9 parts of benzyl alcohol  
100 parts

The above was milled for twelve hours in a ball mill forming a smooth homogeneous assistant dyestuff paste.

EXAMPLE XII

The procedure was the same as in Example X except that 70 parts of Thickener B were substituted for 70 parts of Thickener A. Prints of exceptional brilliancy, levelness and penetration to 20 the reverse side of the fabrics were obtained.

Assistants B, C or D may be substituted for Assistant A with equally good results.

"Sulfanthrene" Orange R Paste may be substituted by the other vat colors mentioned in Example X with equally good results.

EXAMPLE XIII

15 parts of "Sulfanthrene" Blue 2BD Paste (Color Index #1184) were mixed with 30  
60 parts of Thickener A as prepared in Example I  
17 parts of Thickening SBG  
3 parts of sodium hydrosulfite and  
5 parts of a stable emulsion consisting of 35  
45 parts of Turkey red oil  
40 parts of Assistant B  
15 parts of benzyl alcohol  
100 parts

100 parts

The printing paste was heated to 140° F. during 45 which the color was reduced to a considerable extent and then cooled to room temperature. Piece goods containing viscose rayon, Bemberg rayon, cellulose acetate rayon and titanium dioxide delustered rayon were printed with the above printing composition, dried and aged for five minutes 50 at 218° F. After aging, the print was immersed for two minutes in a bath at 130° F. containing 0.5% of sodium perborate and 0.5% of acetic acid. A brilliant blue dyeing of exceptional levelness and penetration on all types of fibers was 55 obtained.

EXAMPLE XIV

5 parts of "Sulfogene" Fast Black CL (In- 60  
docarbon CL) were mixed with  
5 parts of glycerin. To this were added  
80 parts of Thickener B as in Example I and  
10 parts of a stable emulsion consisting of  
20 parts of Turkey red oil  
60 parts of Assistant B  
20 parts of benzyl alcohol  
100 parts

100 parts

Cotton, lustrous rayon, and titanium dioxide delustered rayon were printed with the above printing composition, dried, aged for five min- 75

utes at 214° F. and developed as in Example X. A brilliant and uniform print of excellent penetration to the reverse side of the fabric was obtained.

### EXAMPLE XV

5 parts of Indigosol O4B (leuco sulfuric ester derived from Ciba Blue 2BD—Color Index #1184) were mixed with

10 5 parts of Cellosolve (ethylene-glycol-mono-ethyl-ether)

5 parts of a stable emulsion consisting of

15      10 parts of Turkey red oil

          80 parts of Assistant B

          10 parts of benzyl alcohol

---

          100 parts

20 17 parts of warm water (160° F.) and

      58 parts of neutral starch tragacanth thickening. There were then added

      4 parts of ammonium sulfocyanide (50% solution)

25 4 parts of sodium chlorate (23% solution)

      1 parts of ammonium vanadate (1% solution)

      1 part of ammonia (25% solution)

---

          100 parts

30                    *Starch tragacanth thickening*

      100 parts of wheat starch

      360 parts of gum tragacanth (6% solution)

      540 parts of water

35                    1000 parts

40 Piece goods containing cotton, lustrous and titanium dioxide delustered rayon were printed with the above printing composition, dried and aged for six minutes in the rapid ager. After aging, the material was rinsed, soaped for five minutes at 160° F. in a 0.5% soap solution, rinsed 45 and dried. A brilliant level blue dyeing showing exceptional penetration of color to the reverse side of the fabric was obtained.

EXAMPLE XVI

50 20 parts of "Ponsoi" Violet RRD Paste (Color Index #1104) were mixed with  
 65 parts of Thickener C. To this were added  
 15 parts of a stable emulsion consisting of

55 40 parts of Turkey red oil  
 55 parts of Assistant C  
 5 parts of benzyl alcohol

---

100 parts

60 —  
 100 parts

65 Piece goods containing cotton, viscose rayon, cuprammonium rayon, and ethylene-glycol-di-beta-naphthyl-ether delustered rayon were printed with the above printing composition, dried, aged for two and one-half minutes at 214° F. and developed as in Example X. Although the aging time was curtailed, a bright violet print 70 of exceptional strength, brilliancy and penetration to the reverse side of the fabric was obtained.

Equally satisfactory results may be obtained by employing the triethanolamine salts of the alkyl sulfonic acids included in Assistant C rather than the sodium salts.

### EXAMPLE XVII

20 parts of "Sulfanthrene" Pink FF Paste (Color Index #1211) were mixed with  
70 parts of Thickener C. To this were added  
10 parts of a stable emulsion consisting of 5

30 parts of Turkey red oil  
62 parts of Assistant D  
8 parts of benzyl alcohol  
—  
100 parts

100 parts  
Piece goods containing cotton, cuprammonium rayon, and cellulose acetate fibers were printed with the above printing composition, dried, aged, oxidized, soaped, and finished according to the procedure described in Example X. A brilliant red print was obtained which was sharp in outline and which showed exceptional penetration to the reverse side of the fabric. 15 20

### EXAMPLE XVIII

100 parts of "Sulfanthenene" Orange R Paste 23  
(Color Index #1222) were mixed with  
40 parts of Assistant B and  
20 parts of Turkey red oil

160 parts. There were then evaporated 30  
65 parts of water producing

95 parts. There were then added  
5 parts of benzyl alcohol producing  
100 parts of Assistant "Sulfanethrene" Orange R  
Paste

The above was milled in a colloid mill producing a finely dispersed assistant dyestuff paste adapted for handling in commerce. 40

Instead of "Sulfanthrene" Orange R Paste the following colors were employed with equally good results: "Sulfanthrene" Pink FF Paste (Color Index #1211), "Sulfanthrene" Scarlet Y Paste (Ciba Brown G Paste), "Sulfanthrene" Brown G 4 Paste (Color Index #1212), "Sulfanthrene" Blue 2BD Paste (Color Index #1184), "Ponsol" Jade Green Paste (Color Index #1101), and "Ponsol" Flavone GC Paste (Color Index #1095).

EXAMPLE XIX

100 parts of "Sulfanthrene" Orange R Paste  
(Color Index #1222) were mixed with  
20 parts of Assistant A and  
40 parts of Turkey red oil. 55

160 parts. There were then evaporated  
65 parts of water producing

95 parts. There were then added  
5 parts of benzyl alcohol producing  
100 parts of Assistant "Sulfanethrene" Orange R

Paste. 63  
The above was milled in a colloid mill producing a finely dispersed assistant dyestuff paste adapted for handling in commerce.

Instead of "Sulfanthenrene" Orange R Paste, the colors mentioned in Example X may be employed with equally good results. 70

**EXAMPLE XX**

An easily dispersible vat color powder suitable for printing and dyeing was prepared as follows: 75

2,173,824

7

100 parts of "Sulfanthrene" Blue 2BD Paste  
(Color Index #1184) were mixed with

25 parts of Assistant B  
2 parts of Turkey red oil  
1 part of benzyl alcohol  
36 parts of British gum  
36 parts of sucrose

200 parts

10 Evaporated to dryness and milled the dry mass  
for eight hours in a rod mill, producing an easily  
dispersible powder.

Instead of "Sulfanthrene" Blue 2BD Paste, the  
colors mentioned in Example X may be employed  
15 with equally good results.

EXAMPLE XXI

20 An easily dispersible vat color powder suitable  
for printing and dyeing was prepared as follows:

100 parts of "Sulfanthrene" Pink FF Paste (Col-  
or Index #1211) were mixed with

25 36 parts of Assistant A  
4 parts of Turkey red oil  
2 parts of benzyl alcohol  
5 parts of sodium carbonate

147 parts. Evaporated to dryness and added  
30 31 parts of British gum and  
31 parts of refined glucose

The above was mechanically mixed and then  
milled for ten hours in a ball mill, producing an  
easily dispersible powder. Instead of "Sulfan-  
threne" Pink FF Paste, the colors mentioned in  
35 Example X may be employed with equally good  
results.

This invention has the advantage that vat dye  
40 printing compositions may be easily and econom-  
ically prepared. A further advantage resides in  
the feature that prints characterized by unusual  
penetration to the reverse side of the fabric may  
be easily obtained. A still further advantage re-  
sides in the fact that prints which are free from  
45 specks, mealy or mottled effects may be obtained  
on a commercial scale with facility. The advan-  
tages gained are more noticeably apparent in  
heavy shades than in light shades. This inven-  
tion has the still further advantage that unusual

50

penetration of the dye is obtained in printing  
both lustrous and delustered rayon fabrics.

As many apparently widely different embodi-  
ments of this invention may be made without de-  
parting from the spirit and scope thereof, it will  
be understood that I do not limit myself to the  
specific embodiments thereof except as defined in  
the appended claims.

I claim:

1. A dye composition for printing containing in 10  
addition to a vat dye ingredient, benzyl alcohol  
and at least one sulfonated textile assistant taken  
from the group consisting of Turkey red oil and  
water-soluble sulfates of aliphatic alcohols hav-  
ing from 6 to 12 carbon atoms in which the radi-  
cal attached to the sulfate groups contains not 15  
more than 6 carbon atoms in a chain.

2. A dye composition for printing containing  
in addition to a vat dye ingredient, benzyl alcohol  
and Turkey red oil. 20

3. A dye composition for printing containing  
in addition to a vat dye ingredient, benzyl alcohol  
and a water-soluble sulfate of an aliphatic alco-  
hol having from six to twelve carbon atoms in 25  
which the radical attached to the sulfate group  
contains not more than six carbon atoms in a  
chain.

4. A dye composition of the type set forth in  
claim 3 containing from 0.1 to 20.0% of benzyl  
alcohol. 30

5. A dye composition containing a vat dye,  
from 0.1 to 20% of benzyl alcohol, from 1 to 40%  
of a water-soluble sulfate of an aliphatic alcohol  
having from six to twelve carbon atoms in which  
the radical attached to the sulfate group con- 35  
tains not more than six carbon atoms in a  
straight chain, and from 1 to 40% of Turkey red  
oil.

6. A dyestuff composition especially adapted  
for printing on lustrous and delustered regener- 40  
ated cellulose fibers containing a vat dye ingredi-  
ent, in finely divided form, and from 5 to 20%  
of benzyl alcohol, and at least one sulfonated tex-  
tile assistant taken from the class consisting of  
Turkey red oil and water soluble sulfates of ali-  
phatic alcohols having from 6 to 12 carbon atoms 45  
in which the radical attached to the sulfate  
groups contains not more than 6 carbon atoms in  
a chain.

IVAN F. CHAMBERS. 50

3 - 15  
CERTIFICATE OF CORRECTION.

Patent No. 2,173,824.

September 26, 1939.

IVAN F. CHAMBERS.

It is hereby certified that error appears in the printed specification of the above numbered patent requiring correction as follows: Page 2, second column, line 58, for "reducting" read reducing; page 5, first column, line 5, Example X, for "79 parts" read 70 parts; page 6, first column, line 25, Example XV, for "1 parts" read 1 part; page 7, second column, line 48, claim 6, for the word "carton" read carbon; and that the said Letters Patent should be read with this correction therein that the same may conform to the record of the case in the Patent Office.

Signed and sealed this 14th day of November, A. D. 1939.

(Seal)

Henry Van Arsdale,  
Acting Commissioner of Patents.